

1

3,475,175

**POLYSULFATED ALIPHATIC OR CYCLOALIPHATIC ALCOHOLS AS ANTIFOGGANTS**

James R. King, Jr., Webster, and Thomas E. Whiteley and Louis M. Minsk, Rochester, N.Y., assignors to Eastman Kodak Company, Rochester, N.Y., a corporation of New Jersey

No Drawing. Filed Aug. 19, 1966, Ser. No. 573,479

Int. Cl. G03c 1/34

U.S. Cl. 96—109

18 Claims

**ABSTRACT OF THE DISCLOSURE**

Photographic compositions and photographic elements comprising a silver halide emulsion are stabilized against fog with an effective amount of a water-soluble salt of a polysulfated, aliphatic or cycloaliphatic alcohol containing from 2 to 12 carbon atoms.

This invention relates to new and improved anti-fogants and stabilizers for photographic elements and to photographic silver halide emulsions containing said anti-fogants and stabilizers therein. More particularly, this invention relates to photographic elements and silver halide emulsions containing a salt of a polysulfated, aliphatic or cycloaliphatic alcohol.

During development of a silver halide emulsion, small amounts of silver halide are reduced to metallic silver regardless of whether or not they have been exposed. This reduction of silver ion produces a background fog which is more specifically referred to as chemical fog.

Chemical fog, apparent in most silver halide systems, has been reduced by prior art methods of processing exposed silver halide material in the presence of compounds which restrict development of unexposed silver halide. Such compounds can be incorporated in the silver halide emulsion or in the processing solutions for developing such silver halide emulsions. Compounds which have been found to have a chemical fog inhibiting effect on emulsions which have been subjected to high temperature and high humidity conditions are referred to as emulsion stabilizers. On the other hand, compounds which have been found to have chemical fog inhibiting effects on emulsions which have not been exposed to adverse storage conditions are referred to as antifogants. Although a large number of emulsion stabilizers and antifogants have been used in the prior art, many of these compounds cause undesirable losses in emulsion speed and contrast; others lack adequate compatibility with emulsion gelatin, and still others must be employed in inordinantly high concentrations.

Accordingly, it is an object of our invention to provide novel antifogants and stabilizers for photographic silver halide emulsions.

A further object is to provide a photographic element containing a fog inhibiting compound either in the photographic emulsion or in a layer contiguous thereto.

Still another object is to provide novel antifogants for photographic silver halide emulsions which have little or no effect on the contrast of the processed material.

Still another object is to provide silver halide emulsion stabilizers which maintain sensitivity and fog levels of silver halide emulsions at or near the initial optimum values under conditions of high temperature and humidity.

Other objects will become apparent hereinafter.

The above objects are accomplished by incorporating into the silver halide emulsion of a photographic element or in a layer contiguous to the silver halide emulsion, a fog-stabilizing amount of a water-soluble salt of a poly-

2

sulfated, aliphatic or cycloaliphatic alcohol containing from 2 to 12 carbon atoms. In general, ammonium and alkali metal salts such as sodium, potassium or lithium salts are preferred. Mixtures of alkali metal salts and mixtures of ammonium and alkali metal salts are also quite useful. The salt of the polysulfated, aliphatic or cycloaliphatic alcohol may have hydroxyl or alkyl groups attached thereto and may also contain an oxa group. The ratio of monohydric sulfate groups to the number of carbon atoms in the salt may vary from 1:1 to about 1:3, but is preferably from 1:1 to about 1:2. In the preferred embodiment of the present invention, compounds having from 2 to 6 carbon atoms have been highly effective in inhibiting chemical fog in silver halide emulsions.

Another way to describe the polysulfated salts of the invention is the following formula:



where R is an aliphatic or cycloaliphatic alcohol containing from 2 to 12 carbon atoms, M is an inorganic cation and n is at least 2. Of the inorganic cations that M can represent, ammonium and alkali metals such as sodium, potassium or lithium are preferred. Mixtures of alkali metals and mixtures of alkali metals with ammonium are also quite useful.

The polysulfates of the invention may be prepared by the monohydric sulfation of saturated polyhydroxy compounds such as, for example, the following:

Ethylene glycol  
Diethylene glycol  
Propylene glycol  
Glycerol  
Pentaerythritol  
Dipentaerythritol  
2-methyl-2,4-pentanediol  
1,2,6-hexanetriol  
2,2,5,5-tetramethyl-1,3,4,6-hexanetetrol  
Mannitol  
Dulcitol  
Mannoheptitol  
Inositol  
Sorbitol  
2,7-dimethyloctanediol  
1,2,4-decanetriol  
1,4-cyclohexanediol  
Cyclohexanediethanol, and  
1,2,4,5-tetrahydroxycyclohexane

A convenient method for preparing the compounds of the invention is to heat the polyhydroxy compound with an excess of sulfamic acid in the presence of a solvent, such as hexamethylphosphorotriamide or N,N-dimethylformamide. The product can then be dissolved in water and the pH adjusted for subsequent use with an appropriate base.

The term "polysulfate" as used in this invention refers to compounds containing a plurality of monohydric sulfate groups,  $-OSO_3M$ , where M is an inorganic cation, preferably ammonium or alkali metal or mixtures thereof. Typical examples of polysulfated compounds embraced by our invention are:

Ethylene disulfate ammonium salt  
Ethylene disulfate ammonium-sodium salt  
Diethylene disulfate ammonium salt  
Glycerol trisulfate ammonium salt  
Glycerol trisulfate potassium salt  
Propylene disulfate sodium salt  
Propylene disulfate ammonium salt  
2-methyl-2,4-pentanediol disulfate ammonium salt  
Pentaerythritol tetrasulfate ammonium salt  
Pentaerythritol disulfate ammonium salt  
Dipentaerythritol hexasulfate ammonium-sodium salt

- Mannitol hexasulfate ammonium salt  
 Mannitol tetrasulfate ammonium salt  
 Dulcitol hexasulfate ammonium salt  
 Dulcitol tetrasulfate ammonium-sodium salt  
 Mannoheptitol heptasulfate ammonium salt  
 Mannoheptitol pentasulfate ammonium salt  
 1,2,6-hexanetriol trisulfate ammonium salt  
 1,4-cyclohexanediol disulfate ammonium salt  
 1,2,4,5-tetrahydroxycyclohexane tetrasulfate ammonium sodium salt, and  
 1,2,4,5-tetrahydroxycyclohexane tetrasulfate ammonium salt

The compounds of this invention may be used in any amount which will stabilize the silver halide emulsion against fog. In general, a concentration of the salt in an amount of about 5 g. to about 3 g. per mole of silver in the silver halide emulsion is useful. A preferred concentration for the salt is from about 15 g. to about 30 g. per mole of silver in the silver halide emulsion.

In addition to their excellent fog stabilizing properties, the compounds of the invention tend to increase the speed of the photographic emulsions in which they are incorporated. The increased speed is obtained without adversely affecting other sensitometric properties such as contrast.

The invention can be further illustrated by the following examples or preferred embodiments thereof; although it will be understood that these examples are included merely for purposes of illustration and are not intended to limit the scope of the invention unless otherwise specifically indicated.

The preparation of the fog inhibiting agents in accordance with the invention is exemplified in Examples 1-5.

#### EXAMPLE 1

##### Preparation of ethylene disulfate ammonium salt

Into a 300 ml. three-neck flask, fitted with a magnetic stirrer, a condenser, a thermometer, and a steam bath, were placed 6.2 g. (0.1 mole) of ethylene glycol, 19.4 g. (0.2 mole) of sulfamic acid and 200 ml. of hexamethylphosphorictamide. The mixture was stirred and heated to a homogeneous solution at 100° C. The temperature peaked at 105° C. as the reaction solution became very hazy. Heating was continued for one-half hour, and then the solution was filtered through a Buchner funnel. The clear filtrate was poured into two liters of ethyl acetate. The precipitate was filtered out on a Buchner funnel and washed with 500 ml. of ethyl ether. The product was dried under reduced pressure at 35-40° C. Yield, 20 g.

*Analysis.*—Calcd. for  $C_2H_{12}N_2O_8S_2$ : C, 9.4; H, 4.7; N, 10.9; S, 25.0. Found: C, 10.1; H, 4.7; N, 10.7; S, 23.8.

A solution of 18.6 g. of the dried product in 40 g. of distilled water was prepared and adjusted to pH 7.1 with ten percent ammonium hydroxide. The resulting solution weighed 53.3 g. and contained 31.3 percent solids.

#### EXAMPLE 2

##### Preparation of glycerol trisulfate ammonium salt

Into a 300 ml. three-neck flask, fitted with a magnetic stirrer, a condenser, a thermometer, and a steam bath, were placed 9.2 g. (0.1 mole) of glycerol, 150 ml. of hexamethylphosphorictamide, and 29.1 g. (0.3 mole) of sulfamic acid. The reaction mixture was stirred and heated to a homogeneous solution as the temperature rose and peaked at 113° C. Heating was continued for one-half hour as the temperature dropped to 100° C. The hot hazy reaction solution was filtered through a Buchner funnel with suction.

The clear filtrate was poured into two liters of stirred ethyl acetate. The precipitate was filtered out on a Buchner funnel, washed with 500 ml. of anhydrous ethyl ether, and dried under reduced pressure at 35-40° C. Yield, 31.0 g.

*Analysis.*—Calcd. for  $C_3H_{17}N_3O_{12}S_3$ : C, 9.4; H, 4.5; N, 11.0; S, 25.0. Found: C, 11.2; H, 4.3; N, 10.2; S, 23.8.

A solution of 29.9 g. of the dried product in 75 g. of distilled water was prepared and adjusted to pH 7.1 with ten percent ammonium hydroxide. The resulting solution weighed 104 g. and contained 24.0 percent solids.

#### EXAMPLE 3

##### Preparation of polysulfated dulcitol ammonium salt

- 10 Into a 300 ml. three-neck flask, fitted with a magnetic stirrer, a condenser, a thermometer, and a steam bath, were placed 200 ml. of N,N-dimethylformamide, 9.1 g. (0.05 mole) of dulcitol and 29.1 g. (0.30 mole) of sulfamic acid. The reaction mixture was heated to a homogeneous solution at 86° C. Heating was continued and the temperature peaked at 102° C. as the reaction solution became very hazy. The reaction solution was heated at 95-100° C. for one-half hour, and filtered with suction through a Buchner funnel to yield a clear filtrate.
- 15 20 The filtrate was poured into three liters of stirred methanol and the white precipitate was filtered out on a Buchner funnel and washed with 500 ml. of methanol. The product was dried under reduced pressure at 35-40° C. Yield, 22.8 g.
- 25 25 *Analysis.*—Calcd. for  $C_6H_{32}N_6O_{24}S_6$ : C, 9.5; H, 4.2; N, 11.0; S, 25.2. Found: C, 14.3; H, 5.0; N, 11.8; S, 22.1. A solution of 21.3 g. of the dried product in 60 g. of distilled water was prepared and adjusted to pH 7.1 with ten percent ammonium hydroxide. The resulting solution weighed 77.2 g. and contained 22.6 percent solids.

#### EXAMPLE 4

##### Preparation of polysulfated mannitol ammonium salt

- 30 35 Into a 300 ml. three-neck flask, fitted with a magnetic stirrer, a condenser, a thermometer, and a steam bath, were placed 200 ml. of N,N-dimethylformamide, 9.1 g. (0.05 mole) of mannitol, and 29.1 g. (0.30 mole) of sulfamic acid. The reaction mixture was stirred and heated to a homogeneous solution at 74° C. Heating was continued as the solution became hazy and the temperature peaked at 101° C. The hazy solution was then stirred at 95-100° C. for one-half hour and filtered hot through a Buchner funnel.
- 40 45 The clear filtrate was poured into three liters of stirred methanol and the precipitate was filtered out with suction on a Buchner funnel and washed with 500 ml. of methanol. The product was dried under reduced pressure at 35-40° C. Yield, 21 g.
- 45 50 *Analysis.*—Calcd. for  $C_6H_{32}N_6O_{24}S_6$ : C, 9.5; H, 4.2; N, 11.0; S, 25.2. Found: C, 14.8; H, 5.3; N, 11.6; S, 22.1. A solution of 19.1 g. of the dried product in 60 ml. of distilled water was prepared and adjusted to pH 7.1 with ten percent ammonium hydroxide. The resulting solution contained 28.1 percent solids.

#### EXAMPLE 5

##### Preparation of penetaerythritol tetrasulfate ammonium salt

- 60 65 Into a 300 ml. three-neck flask, fitted with a condenser, a magnetic stirrer, a thermometer, and a heating mantle were placed 13.6 g. (0.1 mole) of pentaerythritol, 48.5 g. (0.5 mole) of sulfamic acid and 200 ml. of N,N-dimethylformamide. The reaction mixture was heated to a homogeneous solution at 75° C. Heating was continued and a white crystalline precipitate separated out at 110° C. The heat was removed and the mixture stirred at ambient temperature for ten minutes.
- 70 75 The precipitate was filtered from the hot N,N-dimethylformamide on a Buchner funnel and washed with 200 ml. of acetone. The crystals were dried under reduced pressure at 45° C. Yield, 39.9 g.
- 75 *Analysis.*—Calcd. for ammonium salt  $C_5H_{24}N_4O_{16}S_4$ : C, 11.4; H, 4.6; N, 10.7; S, 24.4. Found: C, 12.1; H, 5.1; N, 10.9; S, 23.8.

A solution of 15 g. of the dried crystals in 50 ml. of distilled water was prepared and adjusted to pH 0.5 by slurring with Amberlite resin IR 120 (an ion exchange resin comprising polystyrenesulfonic acid manufactured by the Rohm and Haas Company). The resin was filtered off by gravity and the filtrate was adjusted to a pH of 7.1 with ten percent sodium hydroxide. The resulting solution weighed 55.9 g. and contained 19.3 percent solids.

## EXAMPLE 6

Several different compounds of the invention were added to separate portions of a high speed silver bromo-iodide emulsion. Each emulsion sample was coated on a cellulose acetate film support at a coverage of 459 mg. of silver and 1040 mg. of gelatin per square foot. A sample of each film coating was exposed on an Eastman 1B Sensitometer, processed for five minutes in a standard developer (Kodak Developer DK-50), fixed, washed and dried. The photographic results obtained from these tests are listed in Table I.

TABLE I

| Compound                                   | Conc.<br>in<br>g./mole | Fresh |               |       | 2-Week Incubation<br>at 120° F. and 50%<br>Relative<br>Humidity |               |       |
|--------------------------------------------|------------------------|-------|---------------|-------|-----------------------------------------------------------------|---------------|-------|
|                                            |                        | Ag    | Rel.<br>Speed | Gamma | Fog                                                             | Rel.<br>Speed | Gamma |
| Ethylene disulfate ammonium salt           | 9                      | 105   |               | 1.35  | 0.12                                                            | 87            | 1.18  |
| Glycerol trisulfate ammonium salt          | 30                     | 105   |               | 1.33  | 0.10                                                            | 74            | 1.25  |
| Dulcitol hexasulfate ammonium salt         | 30                     | 91    |               | 1.28  | 0.11                                                            | 80            | 1.20  |
| Mannitol hexasulfate ammonium salt         | 30                     | 97    |               | 1.32  | 0.10                                                            | 78            | 1.20  |
| Control                                    |                        | 100   |               | 1.32  | 0.14                                                            | 25            | 0.75  |
| Pentaerythritol tetrasulfate ammonium salt | 30                     | 95    |               | 1.32  | 0.09                                                            | 68            | 1.20  |
| Control                                    |                        | 100   |               | 1.23  | 0.15                                                            | 22            | 0.73  |
|                                            |                        |       |               |       |                                                                 |               | 0.91  |

The results in the above table show that the compounds of the invention prevent the growth of incubation fog when incorporated in photographic emulsions. Further it is seen that these compounds often serve advantageously to increase the emulsion speed while maintaining a stable value for gamma.

The fog-stabilizing effect of the compounds of the invention is surprising and would not have been expected in view of the fact that mono-sulfated alcohols such as Triton 770, and aqueous solution of a sodium salt of an alkylarylpolyether sulfate made by the Rohm and Haas Company, and sodium lauryl sulfate, do not control fog and are essentially inert when incorporated in a photographic emulsion. The following example illustrates this feature.

## EXAMPLE 7

## Comparative test

Samples of Triton 770 and Duponol ME, a sodium lauryl sulfate made by the Du Pont Company, were incorporated in separate portions of photographic emulsion and processed as in Example 6. The results are contained in Table II below.

TABLE II

| Compound   | Conc.<br>in g./<br>mole | Fresh |               |       | 2 Week Incubation at<br>120° F. and 50%<br>Relative Humidity |               |       |
|------------|-------------------------|-------|---------------|-------|--------------------------------------------------------------|---------------|-------|
|            |                         | Ag    | Rel.<br>Speed | Gamma | Fog                                                          | Rel.<br>Speed | Gamma |
| Triton 770 | 12                      | 100   |               | 1.23  | 0.10                                                         | (1)           | (1)   |
| Duponol ME | 12                      | 83    |               | 1.35  | 0.14                                                         | (1)           | (1)   |
| Control    |                         | 100   |               | 1.23  | 0.10                                                         | 15.5          | 0.45  |
|            |                         |       |               |       |                                                              |               | 1.18  |

<sup>1</sup> After two weeks' incubation, the sensitometric strips were uniformly black and it was not possible to distinguish between the individual steps.

Photographic emulsions containing the antifogging and stabilizing agents of the present invention may be sensitized using any of the well-known techniques in emulsion making, for example, by digesting with naturally active gelatin or various sulfur compounds and/or gold compounds. The emulsions may be sensitized with salts of noble metals of Group VIII of the periodic table which have an atomic weight greater than 100. The emulsion

of the invention may be of the surface-sensitive or internally sensitive type. The emulsions may also contain speed-increasing addenda such as quaternary ammonium salts, polyethylene glycols, or thioether sensitizers.

The emulsions of the invention may also contain conventional addenda such as gelatin plasticizers, hardeners and coating aids. These emulsions may be useful in X-ray and other non-optically sensitized emulsions, and may also be used in orthochromatic, panchromatic and infrared sensitive emulsions. The addenda may be added to the emulsion before or after sensitizing dyes, if any, are used. Various silver salts may be used as the sensitive salt, such as silver bromide, silver iodide, silver chloride, or mixed silver halides such as silver chlorobromide or silver bromo-iodide. The emulsions may be used in photographic elements intended for color photography, and thus may contain color-forming couplers, or used as emulsions to be developed by solutions containing couplers or other color-generating materials, or emulsions of the mixed-packet type, as disclosed by Godowsky, U.S. Patent No. 2,698,794,

or emulsions of the mixed-grain type, such as disclosed by Carroll et al., U.S. Patent No. 2,592,243.

The emulsions obtained in accordance with our invention may be used in diffusion transfer processes which utilize the undeveloped silver halide in non-image areas of the negative to form a positive by dissolving the undeveloped silver halide and precipitating it on a silver layer in close proximity to the original silver halide emulsion layer. The emulsions may also be used in diffusion transfer color processes which utilize a diffusion transfer of an imagewise distribution of developer, coupler or dye, from a light-sensitive layer to a second layer, while the two layers are in close proximity to one another.

A wide variety of emulsion vehicles and dispersing agents for silver halide grains may be employed singly or in combination with each other, for example, gelatin, colloidal albumen, cellulose derivatives and synthetic resins, such as polyvinyl compounds. Examples of typical colloids which may be used are poly(vinyl alcohol), hydrolyzed poly(vinyl acetate), hydrolyzed cellulose ester, water-soluble ethanolamine cellulose acetate, polyacrylamide, copolymers having a combined acrylamide content of 3-60 percent, copolymers of alkyl acrylate and acrylic acid, a vinyl alcohol copolymer containing urethane carboxylic acid groups or containing cyano-acetyl groups, or polymeric material which results from polymerizing a protein or saturated acrylated protein with a monomer having a vinyl group such as disclosed by Ellingsworth, U.S. Patent 2,852,382. Such polymeric addenda may be employed as latices of hydrosols in the preparation of the photographic emulsions of our invention.

The antifogging agents of our invention may be incorporated to advantage during manufacture in silver halide emulsions representing the variations described above. Moreover, fog control in binderless silver halide films prepared by vapor deposition of silver halide on a suitable support may be achieved by coating the antifogging agents of the invention over the vapor-deposited layer of silver halide.

Although the invention has been described in considerable detail with reference to certain embodiments thereof, it will be understood that variations and modifications can be effected without departing from the spirit and

scope of the invention as described hereinabove and as defined in the appended claims.

We claim:

1. A composition comprising a photographic silver halide emulsion containing a fog-stabilizing amount of a water-soluble salt having the formula:



where R is a residue of a polyhydroxy aliphatic or cycloaliphatic alcohol containing from 2 to 12 carbon atoms and having at least two of said hydroxy groups each replaced by a monohydric sulfate group, M is an inorganic cation and n is at least 2.

2. The composition of claim 1 wherein said salt is present in an amount of about 5 to about 30 grams per mole of silver in said silver halide emulsion.

3. The composition of claim 1 wherein each M is ammonium or an alkali metal.

4. The composition of claim 1 wherein said salt is ethylene disulfate ammonium salt.

5. The composition of claim 1 wherein said salt is glycerol trisulfate ammonium salt.

6. The composition of claim 1 wherein said salt is dulcitol hexasulfate ammonium salt.

7. The composition of claim 1 wherein said salt is 25 mannitol hexasulfate ammonium salt.

8. The composition of claim 1 wherein said salt is pentaerythritol tetrasulfate ammonium-sodium salt.

9. A photographic element comprising a support coated with a silver halide emulsion, said element containing a 30 for-stabilizing amount of a water-soluble salt having the following formula:



where R is a residue of a polyhydroxy aliphatic or cycloaliphatic alcohol containing from 2 to 12 carbon atoms and having at least two of said hydroxy groups each replaced by a monohydric sulfate group, M is an inorganic cation and n is at least 2.

5 10. The photographic element of claim 9 wherein said salt is present in an amount of about 5 to about 30 grams per mole of silver in said silver halide emulsion.

11. The photographic element of claim 9 wherein each M is ammonium or an alkali metal.

12. The photographic element of claim 9 wherein said salt is ethylene disulfate ammonium salt.

13. The photographic element of claim 9 wherein said salt is glycerol trisulfate ammonium salt.

14. The photographic element of claim 9 wherein said salt is dulcitol hexasulfate ammonium salt.

15. The photographic element of claim 9 wherein said salt is mannitol hexasulfate ammonium salt.

16. The photographic element of claim 9 wherein said salt is pentaerythritol tetrasulfate ammonium-sodium salt.

17. The photographic element of claim 9 wherein said salt is present in said silver halide emulsion.

18. The photographic element of claim 9 wherein said salt is present in a layer contiguous to said silver halide emulsion.

#### References Cited

##### UNITED STATES PATENTS

3,392,023 7/1968 Burness ----- 96-109 X  
3,396,028 8/1968 Humphlett ----- 96-109

NORMAN G. TORCHIN, Primary Examiner

R. E. FICHTER, Assistant Examiner

UNITED STATES PATENT OFFICE  
CERTIFICATE OF CORRECTION

Patent No. 3,473,175 Dated October 23, 1969

Inventor(s) James R. King et al

It is certified that error appears in the above-identified patent and that said Letters Patent are hereby corrected as shown below:

Claim 7, line 1 -- "2 g." per mole should be "2 g. per mole"

Claim 1, line 5 -- "salt" should be "a salt"

Claim 9, line 31 -- "for" should be "a" "for"

Claim 11, line 5 -- "photographic" should be "photographic"

SIGNED AND  
SEALED  
MAY 12 1970

(SEAL)

Attest:

Edward M. Fletcher, Jr.

Attesting Officer

WILLIAM E. SCHUYLER, JR.  
Commissioner of Patents